

(No Model.)

J. EVETTS & F. C. SCHURZ.  
PROCESS OF ANNEALING METAL CASTINGS.

No. 570,919.

Patented Nov. 10, 1896.



Witnesses:

Olym Bishop  
Selden Fish

Inventors:

James Evetts  
Francis C. Schurz

# UNITED STATES PATENT OFFICE.

JAMES EVETTS AND FRANCIS C. SCHURZ, OF CHICAGO, ILLINOIS.

## PROCESS OF ANNEALING METAL CASTINGS.

SPECIFICATION forming part of Letters Patent No. 570,919, dated November 10, 1896.

Application filed July 11, 1896. Serial No. 598,788. (No specimens.)

*To all whom it may concern:*

Be it known that we, JAMES EVETTS, a subject of the Queen of Great Britain, and FRANCIS C. SCHURZ, a citizen of the United States, 5 residing at Chicago, in the county of Cook and State of Illinois, have invented a certain new and useful Improvement in Processes of Annealing Metal Castings, of which the following is a full, clear, concise, and exact description, reference being had to the accompanying drawing, forming a part of this specification.

Our invention relates to a process of annealing metal castings, and has for its object 15 to provide means for annealing or decarbonizing metal castings, as, for instance, steel castings, in shorter space of time and with less application of heat than heretofore.

The process of our invention may be generally described as consisting in enveloping the castings to be annealed in fibrous or finely-divided asbestos, which is preferably tightly packed about the castings in a porous or perforated chamber, whereupon the whole is introduced into the annealing-furnace and subjected to an annealing heat for a period of, say, twenty-four hours, when it is withdrawn therefrom and allowed to cool slowly, the process being thus completed. The asbestos may 30 be slightly moistened when packing to secure flexibility.

The advantages of this system are as follows: The thorough enveloping of the casting in the non-conducting material secures a 35 more even and regular heating; also the asbestos fiber, being in intimate contact with the surfaces of the metal, precludes the possibility of an oxid scale or crust forming on said surfaces, thereby allowing the atmospheric oxygen free and uninterrupted access to the same. By this means the decarbonizing process is carried on with much greater speed, and the possibility of breaking or cracking the casting is greatly decreased.

The packing of asbestos fiber having once 45 admitted the heat, retains it for a sufficient period of time to insure very gradual cooling of the casting.

The rough scaly surfaces which are present in castings annealed after the ordinary 50 method are totally obviated by our process of annealing, as when the protecting fiber is removed the castings come out with clean and smooth surfaces.

In the drawing, *a* represents a bar of cast- 55 steel, around which is packed the asbestos fiber *b*, contained in the iron box *c*, said asbestos fiber being first moistened to secure flexibility, and afterward tamped thoroughly in. The box *c* has perforations *d d* drilled in 60 its walls to admit of a free circulation of air and escape of vapor. The box is then closed, and the whole introduced into the annealing-furnace, where it is allowed to remain for a period of, say, twenty-four hours, when it is 65 withdrawn and allowed to cool, the process thereupon being completed.

A saving of time varying from seven to ten days is thus effected by the process of our invention over the methods heretofore in use. 70

Having thus described our invention, what we claim as new, and desire to secure by Letters Patent, is—

The process of annealing metal castings, 75 which consists in enveloping the castings to be annealed in fibrous or finely-divided asbestos, which is tightly packed about the castings in a perforated or porous chamber or casing, the whole being exposed to an annealing heat and allowed to slowly cool, substantially as described.

In witness whereof we hereunto subscribe our names this 8th day of July, A. D. 1896.

JAMES EVETTS.

FRANCIS C. SCHURZ.

Witnesses:

ELMER BISHOP,  
SELDEN FISH.